

## UNITED STATES PATENT OFFICE

2,413,428

## LUBRICATION OF TEXTILE FIBERS

Howard J. Billings, South Acton, Mass., assignor  
to Monsanto Chemical Company, St. Louis, Mo.,  
a corporation of Delaware

No Drawing. Application November 3, 1943,  
Serial No. 508,858

9 Claims. (Cl. 57—164)

1

This invention relates to a method for lubricating textile fibers.

In the processing of fibers for the manufacture of textile products, it is customary to use a lubricant for the fibers. The lubricant has two principal functions—first, it lubricates the fibers during the various processing steps, thereby minimizing fiber breakage especially in opening processes such as carding; and second, it acts as an adhesive in that it prevents fly in carding operations and also promotes cohesion of the fibers into a loose sliver, thereby facilitating condensing, drafting, and spinning. After the lubricant has performed its functions, it is usually removed from the fibers by scouring.

While there are a number of fiber lubricants on the market, the lubricants most extensively used are olive oil, certain types of mineral oils, both uncompounded and compounded (i. e., blended or specially processed), and also various glycerides such as lard oil, as well as some proprietary glycerides. These lubricants, however, have been found unsuitable in varying degrees with respect to either scourability, odor, price, lubricating properties, deterioration on aging, dyeing properties of the fibers, or other characteristics.

It is accordingly a principal object of this invention to provide a class of compounds which are definitely superior in lubricating and related properties to known lubricants and lack their disadvantages. Other objects will be clear from the following disclosure.

The compounds which I have found suitable for the purposes of this invention are the alkali and alkylolamine salts of alkyl phosphoric acids, and specifically the named salts of such acids in which the alkyl group contains not more than five carbon atoms. These compounds are all thoroughly water-soluble, and markedly hygroscopic; their water-solutions are fluid at operating conditions of fiber processing, which are in the general range of 40% to 65% relative humidity at 70° F. They manifest a pH value in water solution which is either substantially neutral or moderately on the alkaline side of neutrality; they are not so acidic as to be hazardous to the operators or corrode the machinery, nor so alkaline as to injure the fibers. The resulting pH should in general be not lower than 5 nor higher than 11, and the preferable working range is between pH=6 and pH=10. Films of water-solutions of these materials do not appear to penetrate the fibers; hence they are effective lubricants. They are substantially without odor, and do not develop odor on standing nor under any conditions of plant operation. They are stable to temperatures even up to the boiling point of their water solutions. Either in water solution or alone, they are non-inflammable, non-volatile, and non-cor-

2

rosive, and are non-toxic to the operators. Their viscosity in water-solution may be varied within a wide range, sufficient to meet any fiber-lubrication requirements. Their price is within the range of the price of ordinary lubricants.

The advantages of my preferred class of lubricants are clear from the foregoing discussion. Certain of these advantages, however, will now be particularly pointed out. In the first place, these compounds, being water-soluble are readily scoured out with water. No soaps or other special materials are necessary for this purpose—thus differing markedly from the procedure with conventional lubricants. Furthermore, since these compounds are positively hygroscopic, they do not dry out, even when in very thin films, under the normal temperature and humidity conditions of the mill operations. Furthermore, the substantial neutrality or moderate alkalinity of the water-solutions of these compounds assures the absence of alkalies strong enough to damage certain types of fibers—particularly animal fibers such as wool.

Included among the compounds of this invention are both the sodium and potassium salts of the alkyl phosphoric acids, e. g., sodium (or potassium) methyl phosphate, sodium (or potassium) ethyl phosphate, sodium (or potassium) amyl phosphate, and mixtures and mixed compounds of these and related compounds of this class, such as sodium potassium methyl phosphate, sodium potassium ethyl phosphate, sodium potassium amyl phosphate and the sodium (or potassium) salts of the mixture of alkyl phosphoric acids obtained by reacting three mols of a suitable alcohol with one mol of phosphorus pentoxide. Moreover, I may use to advantage the alkylolamine salts of alkyl phosphoric acids, such as the di or tri methanol or ethanol amine salts of methyl or ethyl phosphoric acids. The criteria of operability of such compounds has already been set forth—e. g., they must be water-soluble, positively hygroscopic, have a pH in water-solution which is not high enough to injure the fiber (preferably not over 10), and be effective lubricants. Specifically, the specific compounds just mentioned have pH values in water-solution ranging between 7 and 8 in the dilutions used (e. g., 50%). They are furthermore, stable under all operating conditions, and even up to at least their boiling point in water solution.

In carrying out the process of this invention in connection with the lubrication of fibers, I first prepare a water-solution of one or more materials of the class of lubricants herein defined, and then apply it to the fibers in any suitable manner, as by spraying. As a specific example, using the process of lubricating worsteds for an illustration, I make up a water-solution of sodium potassium ethyl phosphate having between

40% and 50% water, by weight, and apply the same to the stock. The stock is then passed through the usual textile operations of spinning, weaving, etc., and, when the lubricant has finished performing its functions, it may be removed by merely washing in water. During the mill operations and while the lubricant is on the fibers, the humidity of the surrounding air should not go (at least for any length of time) appreciably below the point at which the lubricant begins to lose water faster than it takes it up due to its hygroscopic properties. For sodium potassium ethyl phosphate this point is at about 40% relative humidity at 70° F. for the best results, but may be even as low as about 25% if not maintained that low for a prolonged period—i. e., during an appreciable portion of the time that the lubricant is on the fibers. If, however, the lubricant should be allowed to dry out, as when the lubricated stock is, for example, stored at too low a relative humidity, the lubricant can be readily returned to its proper condition by putting it into the presence of an atmosphere of proper relative humidity—e. g., 50% or over at 70° F.

Similar procedure is followed in using the other compounds in the class of lubricants herein defined. This procedure may be modified as desired, within the scope of this invention, for specific purposes. Other fibers than wool may be effectively lubricated by the procedure of this invention. Such lubrication is particularly desirable in connection with the processing of animal fibers generally, but is not limited thereto.

Although the products referred to herein have been described as lubricants, they do not act as lubricants in the same manner or in the same sense as the oily materials of the prior art. Thus, their lubricating action is primarily due to the maintenance of water wetness and the elimination of static rather than to any tendency toward or characteristic of oiliness.

This application is a continuation-in-part of application Serial No. 369,713, filed December 12, 1940.

What I claim is:

1. As a stage product in the manufacture of textile products, a textile fiber having a fluid coating which comprises a substance selected from the group consisting of alkali and alkyloamine salts of alkyl phosphoric acid, in which the alkyl group has between one and five carbon atoms, said coating manifesting a pH value between 5 and 11 when in approximately an equal weight of water and maintaining its fluidity at relative humidities not substantially lower than 40% at 70° F.

2. Textile fibers which have been coated with a lubricant and anti-static composition containing as its essential lubricant and anti-static component an aqueous solution of an alkali alkyl phosphate, in which the alkyl group has between one and five carbon atoms, said coated fibers being substantially free of static and maintaining water wetness at relative humidities not substantially lower than 40% at 70° F.

3. Textile fibers which have been coated with a lubricant and anti-static composition containing as its essential lubricant and anti-static component an aqueous solution of an alkyloamine alkyl phosphate, in which the alkyl group has between one and five carbon atoms, said coated fibers being substantially free of static and main-

taining water wetness at relative humidities not substantially lower than 40% at 70° F.

4. As a stage product in the manufacture of textile products, a textile fiber having a fluid coating which comprises sodium potassium ethyl phosphate, said coating manifesting a pH value between 6 and 10 when in approximately an equal weight of water and maintaining its fluidity at relative humidities not substantially lower than 40% at 70° F.

5. As a stage product in the manufacture of textile products, a textile fiber having a fluid coating which comprises sodium potassium amyl phosphate, said coating manifesting a pH value between 6 and 10 when in approximately an equal weight of water and maintaining its fluidity at relative humidities not substantially lower than 40% at 70° F.

6. As a stage product in the manufacture of textile products, a textile fiber having a fluid coating which comprises triethanolamine ethyl phosphate, said coating manifesting a pH value between 6 and 10 in approximately an equal weight of water and maintaining its fluidity at relative humidities not substantially lower than 40% at 70° F.

7. The method of treating textile fibers to render them more amenable to textile processing steps such as carding, condensing, drafting and spinning which comprises applying to said fibers at some stage prior to spinning a fluid coating which consists essentially of water and a substance selected from the group consisting of alkali and alkyloamine salts of alkyl phosphoric acid, in which the alkyl group has from 1 to 5 carbon atoms, said coating being capable of maintaining its fluidity at relative humidities not substantially lower than 40% at 70° F., whereby said treated fibers are maintained substantially free of static during said processing steps.

8. The method of spinning fibers which comprises applying to said fibers at some stage prior to spinning a fluid aqueous coating in the form of a thin film consisting essentially of water and a substance selected from the group consisting of alkali and alkyloamine salts of alkyl phosphoric acid, in which the alkyl group has from 1 to 5 carbon atoms, and then spinning the resulting fibers, the atmosphere surrounding the fibers being maintained at a relative humidity not substantially lower than 40% at 70° F. from the time said coating is applied until the completion of the spinning, whereby said coating is maintained in a substantially water-wet state and said fibers are maintained substantially free of static.

9. The method of spinning fibers which comprises applying to said fibers at some stage prior to spinning a fluid aqueous coating in the form of a thin film consisting essentially of water and a substance selected from the group consisting of alkali and alkyloamine salts of alkyl phosphoric acid, in which the alkyl group has from 1 to 5 carbon atoms, spinning the resulting fibers and removing said coating after the spinning is completed, the atmosphere surrounding the fiber being maintained at a relative humidity not substantially lower than 40% at 70° F. from the time said coating is applied until the completion of the spinning, whereby said coating is maintained in a substantially water-wet state and said fibers are maintained substantially free of static.

HOWARD J. BILLINGS.